

## 1

3,390,984

**HIGH-TEMPERATURE DUCTILE ALLOYS**  
 Clayton D. Dickinson, Port Washington, and Sam Friedman, Great Neck, N.Y., assignors to General Telephone and Electronics Laboratories, Inc., a corporation of Delaware  
 No Drawing. Filed Mar. 29, 1965, Ser. No. 443,692  
 6 Claims. (Cl. 75—176)

**ABSTRACT OF THE DISCLOSURE**

A group of tungsten-base alloys containing 0.03 to 0.4% thorium, 0.002 to 0.03% carbon and up to 7.0% rhenium. These alloys exhibit low ductile-to-brittle transition temperatures, high strength at elevated temperatures and high recrystallization temperatures.

This invention relates to tungsten-base alloys characterized by high strength at elevated temperatures and to tungsten-base alloys which combine high elevated temperature strength with a low ductile-to-brittle transition temperature.

The tungsten-base alloys of the present invention contain rhenium, carbon and thorium. As is well known, the addition of rhenium to tungsten produces alloys having reduced ductile-to-brittle transition temperatures but the scarcity and high cost of rhenium have limited the use of these materials for many applications such as sheet, tubing and other wrought forms. Accordingly, it is an object of the invention to provide alloys which employ relatively small amounts of rhenium yet have low ductile-to-brittle transition temperatures, high strength at elevated temperatures and high recrystallization temperatures.

In the present invention, tungsten-base alloys are provided which contain up to 7.0% rhenium, 0.002% to 0.03% carbon and between 0.03% to 0.4% thorium. (All percentages given are by weight.) In addition, alloys have been produced which contain only tungsten, carbon and thorium, these alloys having high elevated temperature strength although they lack ductility at low temperatures. By varying the constituents within the specified ranges the best combination of mechanical properties and ease of fabricability may be obtained for a given application.

Compared with unalloyed tungsten made by the same process the present alloys are generally stronger at 1650° C., have higher recrystallization temperatures and, when rhenium is incorporated, are ductile at lower temperatures. In particular, a number of the alloys in the system are completely ductile at room temperature or below. For example, the alloys exhibit ultimate tensile strength at 1650° C. in the range 23,000 p.s.i. to 43,000 p.s.i. as compared to 13,000 p.s.i. for unalloyed tungsten. The ductile-

10

15

20

25

30

35

40

45

50

55

## 2

to-brittle transitions for rhenium containing alloys occur in the range from —25° C. to +100° C. in comparison with 175° C. for unalloyed tungsten. The recrystallization temperatures for unalloyed tungsten is between 1450° C. and 1500° C. whereas the present alloys have recrystallization temperatures in the range 1600° C. to 1875° C. The high strengths and high recrystallization temperatures obtained in these tungsten-base alloys is believed due to the formation during fabrication of uniformly dispersed particles of thorium carbide having particle sizes predominantly in the range 200 to 1000 Angstroms.

**EXAMPLE I**

Elemental powders of thorium, carbon, rhenium and tungsten were blended to form a uniform mixture which was then subjected to a pressure of approximately 50,000 pounds per square inch to form a billet. The billet was next sintered at a temperature of about 2350° C. for approximately 4 hours to mutually diffuse the different ingredients thereby forming a solid solution of thorium and rhenium in tungsten, the carbon probably being partitioned between tungsten carbide and a solid solution of carbon in tungsten. The billet was then fabricated by forging at a temperature of approximately 1850° C. from 0.5 inch to 0.3 inch thick followed by rolling at a temperature of about 1550° C. to form sheets having a thickness of approximately 0.040 inch. During the fabrication process, carbon precipitates as finely dispersed thorium carbide. While a powder metallurgy process was used in forming the sheets, it shall be understood that the alloys may also be consolidated by other suitable processes such as vacuum arc-casing. Fabrication may be accomplished by other techniques such as extruding, forging or drawing to produce the desired wrought form.

Measurements of ultimate tensile strength, recrystallization temperature and ductile-to-brittle transition temperature were carried out for a number of alloys. The recrystallization temperature was established by determining at what temperature the alloy must be heated for one hour before the fibrous structure completely disappears and recrystallization is essentially complete. The transition from ductile-to-brittle behavior, which occurs over a range of temperatures, was measured by attempting to bend specimens 1 inch long by  $\frac{3}{8}$  inch wide by 0.04 inch thick over a radius four times the thickness of the sheet through a 105° angle at several temperatures and determining the minimum temperature at which the sample cracked after a small but perceptible amount of bending (nil ductility temperature) and the minimum temperature at which the sample bent 105° without cracking (ductility temperature).

Characteristics of the alloys at different compositions are shown in Table I. A dash in the table indicates that the listed property was not measured for that sample.

TABLE I

| Alloys, Percent by Weight |     |       |         | Ultimate Tensile Strength at 1,650° C. (p.s.i.) | Ductile-to-Brittle Transition Temp. (° C.) |                 | One Hour Recrystallization Temp. (° C.) |
|---------------------------|-----|-------|---------|-------------------------------------------------|--------------------------------------------|-----------------|-----------------------------------------|
| Th                        | Re  | C     | W       |                                                 | Nil Det. Temp.                             | Ductility Temp. |                                         |
| 0.08                      | 5.0 | 0.012 | Balance | 32,000                                          | 65                                         | 100             | 1,700-1,750                             |
| 0.10                      | 5.0 | 0.019 | Balance | —                                               | —50                                        | —25             | —                                       |
| 0.15                      | 1.0 | 0.010 | Balance | 41,000                                          | 10                                         | 25              | 1,800-1,825                             |
| 0.15                      | 3.0 | 0.009 | Balance | 39,000                                          | 25                                         | 100             | 1,725-1,750                             |
| 0.15                      | 7.0 | 0.004 | Balance | 23,000                                          | <10                                        | —               | 1,600-1,625                             |
| 0.35                      | 5.0 | 0.003 | Balance | 35,000                                          | —25                                        | 10              | 1,650-1,675                             |

**3**  
**EXAMPLE II**

An alloy consisting of thorium, carbon and tungsten was prepared by the method described for the alloy of Example I. Table II gives the characteristics of various compositions of this alloy.

TABLE II

| Alloys, Percent by Weight |       |         | Ultimate Tensile Strength at 1,650° C.<br>(p.s.i.) | Ductile-to-Brittle Transition Temp. (° C.) |                 | One Hour Recrystallization Temp. (° C.) |
|---------------------------|-------|---------|----------------------------------------------------|--------------------------------------------|-----------------|-----------------------------------------|
| Th                        | C     | W       |                                                    | Nil Duct. Temp.                            | Ductility Temp. |                                         |
| 0.03                      | 0.004 | Balance | 37,000                                             | —                                          | —               | —                                       |
| 0.13                      | 0.029 | Balance | 43,000                                             | —                                          | —               | 1,850-1,875                             |
| 0.13                      | 0.024 | Balance | 43,000                                             | —                                          | —               | 1,850-1,875                             |

From these results it is apparent that those alloys containing at least 1% rhenium exhibit high strength at elevated temperatures and are ductile at low temperatures. Thorium-carbon-tungsten alloys without rhenium have high elevated temperature strength but are not ductile at low temperatures. All of the disclosed alloys have high recrystallization temperatures as compared to unalloyed tungsten. For applications where a high melting point is desired, the composition containing the minimum alloying ingredients consistent with desired mechanical properties have been found most suitable.

As many changes could be made in the above described compositions it is intended that all matter contained therein shall be interpreted as illustrative and not in a limiting sense.

What is claimed is:

1. An alloy consisting essentially of 0.03% to 0.4% thorium, 0.003% to 0.03% carbon, and up to 7.0% rhenium, the balance consisting of tungsten.
2. An alloy consisting essentially of 0.08% to 0.4% thorium, 0.003% to 0.19% carbon, and 1.0% to 7.0% rhenium, the balance consisting of tungsten.
3. A tungsten-base alloy characterized by high strength at elevated temperatures and a low ductile-to-brittle transition temperature consisting essentially of about 0.15%

thorium, 0.01% carbon and 1.0% rhenium, the balance consisting of tungsten.

4. A tungsten-base alloy characterized by high strength at elevated temperatures consisting essentially of 0.03% to 0.13% thorium and 0.004% to 0.3% carbon, the balance consisting of tungsten.

5. A tungsten-base alloy characterized by high strength at elevated temperatures and low ductile-to-brittle transition temperature consisting essentially of from 0.10% to 0.15% thorium, 1% to 7% rhenium, and 0.004% to 0.019% carbon, the balance consisting of tungsten.

6. An alloy consisting essentially of 0.03% to 0.04% thorium, 0.003% to 0.03% carbon and up to 7% rhenium, the balance consisting of tungsten, said alloy containing uniformly dispersed particles of thorium carbide having particle sizes predominantly in the range 200 to 2000 angstroms.

**References Cited**

**UNITED STATES PATENTS**

|           |         |                        |        |
|-----------|---------|------------------------|--------|
| 2,580,171 | 12/1951 | Hagglund et al. -----  | 75—124 |
| 3,116,145 | 12/1963 | Semchyshen -----       | 75—176 |
| 3,236,699 | 2/1966  | Pugh et al. -----      | 75—176 |
| 3,243,291 | 3/1966  | Dickinson et al. ----- | 75—176 |

**OTHER REFERENCES**

Nb, Ta, Mo and W, Quarrell, Elsevier Publishing Co., New York, 1961, relied on pp. 321 and 347-361.

CHARLES N. LOVELL, *Primary Examiner.*